# EUROPEAN PATENT SPECIFICATION

(11) **EP 2 406 423 B1**
(45) Date of publication and mention of the grant of the patent: **21.11.2012**
(21) Application number: 10706576.5
(22) Date of filing: 17.02.2010
(51) Int. Cl.: D06M 15/643, D06M 11/77, D06M 13/184, D06M 11/78, D06M 13/188, D06M 13/203, C11D 3/00

(54) **FABRIC TREATMENT COMPOSITION AND METHOD**
GEWEBEBEHANDLUNGSZUSAMMENSETZUNG UND -VERFAHREN
COMPOSITION ET PROCÉDÉ DE TRAITEMENT D'UN TISSU

(30) Priority: 09.03.2009 IN MU05082009
(43) Date of publication of application: 18.01.2012
(73) Proprietor: Unilever NV, 3013 AL Rotterdam (NL); Unilever PLC, London, Greater London EC4Y 0DY (GB)
(72) Inventor: BHATTACHARYA, Arpita, Bangalore 560 066 (IN); PANCHANATHAN, Anandh, Bangalore 560 066 (IN); JAYARAMAN, Suresh, Sambamurthy, Bangalore 560 066 (IN); CHATTERJEE, Debsoree, Bangalore, 560 066 (IN)
(74) Representative: Chisem, Janet
(86) International application number: PCT/EP2010/051963
(87) International publication number: WO 2010/102882

(56) References cited:
- EP-A1- 0 244 500
- GB-A- 2 388 610

## Description

### TECHNICAL FIELD

The present invention relates to a fabric treatment composition and a method of treatment of fabric.

### BACKGROUND AND PRIOR ART

Any discussion of the prior art throughout the specification should in no way be considered as an admission that such prior art is widely known or forms part of the common general knowledge in the field.

Conventional cleaning methods are directed towards effective cleaning of soils from the fabrics. Some cleaning formulations include soil release agents that make it easier for oily soils to be cleaned from fabrics. However, conventional cleaning formulations do not help much in reducing subsequent post-wash soiling of the fabric.

On the other hand, various industrial treatments for fabric modification are known to render the fabric hydrophobic by lowering surface energy or by providing a surface texture with optimum roughness or by a combination of both the approaches. The fabric modification of this type is normally carried out during textile manufacture and involves elaborate processes using expensive chemicals such as fluoropolymers. Further, these processes are relatively difficult to be conveniently used in household.

Thus there is an unfulfilled need for a fabric treating method that can be used in household for reduction of subsequent soiling of fabrics.

One such method, disclosed in our pending application 1691/MUM/2007 (Hindustan Unilever Limited), is a multi-step method of treating a fabric with a compound of alkaline earth metal, titanium or zinc, with a water-soluble compound of aluminium, and with C8-C24 soap, in presence of an aqueous carrier. However, the multi-step method disclosed therein is relatively less convenient and relatively less user-friendly. Furthermore, for the method to be used effectively, it must be communicated to the end-user to apply the ingredients to the fabric In a stepwise manner. End-users may not have adequate level of education to follow the instructions correctly and there is a need for a single step method for imparting hydrophobicity and reducing subsequent cleaning.

EP-A1-0 244 500 discloses a water repellent composition being liquid at room temperature, which comprises a silicone oil and a substantially non-volatile paraffinic oil or low molecular weight hydrocarbon resin, wherein the separation index of the paraffinic oll or low molecular weight hydrocarbon resin to the silicone oil is at most 0.4.

It is an object of the present invention to overcome or ameliorate at least one of the disadvantages of the prior art, or to provide a useful alternative.

One of the objects of the present invention is to provide a method and a composition for treating a fabric to render the fabrics relatively more hydrophobic.

Another object of the present invention is to provide a method and a composition for treating a fabric to impart relatively better stain-resistance to the fabric.

Present inventors have surprisingly found that a composition comprising clay, silicone oil and fatty acid when contacted with a fabric in presence of water under specific pH conditions, renders the fabric hydrophobic.

### SUMMARY OF THE INVENTION

According to a first aspect of the present invention there is provided a fabric treatment composition comprising clay, silicone oil, and fatty acid, characterized in that
a. the composition comprises at least 30% by weight of clay, and
b. pH of the composition is less than or equal to 6.

According to a second aspect of the present invention there is provided a method of treatment of fabric comprising a step of contacting the fabric with the fabric treatment composition of the first aspect in presence of water.

### DETAILED DESCRIPTION OF THE INVENTION

### The Fabric

The fabric that can be treated includes synthetic as well as natural textiles. Fabrics may be made of cotton, polycotton, polyester, silk or nylon. It is envisaged that the method of the present invention can be used to treat garments and other clothing and apparel materials that form typical wash-load in household laundry. The household materials that can be treated according to the process of the present invention include, but are not limited to, bedspreads, blankets, carpets, curtains and upholstery. Although the process of the present invention is described primarily for treatment of a fabric, it is envisaged that the process of the present invention can be advantageously used to treat other materials such as jute, denim and canvass. It is envisaged that the process of the present invention can be used to treat articles such as shoes and jackets.

### Clay

The fabric treatment composition comprises at least 30% by weight of clay. The clay is preferably from 30% to 90%, more preferably from 50% to 90% by weight and most preferably from 60% to 85% by weight of the fabric treatment composition.

Although any type of clay can be used, it is preferred that the clay is a 2:1 clay. 1:1 clays that can be used include kaolinite, dickite, halloyside, nacrite, chrysolite, lizardite, and amesite. Preferred 2:1 clays are montmorrilonite, bentonite, and smectite.

### Silicone Oil

The silicone oil is preferably from 3% to 50%, more preferably from 3% to 30% by weight and most preferably from 5% to 10% by weight of the fabric treatment composition. Preferred silicone oil is polydimethylsiloxane.

Some examples of commercially available silicone oils that can be used include Q2-1607 (ex Dow Corning), 1107 (ex Dow Corning), SF8417 (ex Dow Corning), Q2-8166 (ex Dow Corning), 2-8630, Q2-8460 (ex Dow Corning), 3-0213 (ex Dow Corning), 2-8040 (ex Dow Corning) and ARA-222 (ex Dyetech, Inc), SM2125 (ex Momentive performance materials), SMW32 (ex Momentive performance materials), SM2059 (ex Momentive performance materials) and AN101 (ex Resil), AE104 (ex Resil) and AE112 (ex Resil).

### Fatty Acid

The fatty acid is preferably from 5% to 50%, more preferably from 5% to 30% by weight and most preferably from 5% to 20% by weight of the fabric treatment composition.

The number of carbon atoms in the fatty acid is preferably from 8 to 50, more preferably from 10 to 48, most preferably from 12 to 22.

Although both saturated and unsaturated fatty acids can be used, it is preferred that the fatty acid is a saturated fatty acid. The saturated fatty acid is preferably selected from lauric acid, myristic acid, stearic acid, palmitic acid, or mixtures thereof.

Examples of unsaturated fatty acids include oleic acid, linoleic acid, linoleinic acid, ricinoleic acid, elaidic acid, petroselenic acid, erucic acid, palmitoleic acid, myrostoleic acid, and 12-hydroxyoleic acid.

Fatty acid may be directly added to the composition, Alternatively, it is envisaged that a corresponding fatty acid soap and an inorganic or organic acid are added to the composition for in situ generation of the fatty acid in the composition.

Preferably the mass ratio of clay to fatty acid is greater than 1.

### pH Of The Fabric Treatment Composition

pH of the fabric treatment composition refers to pH of a mixture obtained by adding 1 part of the fabric treatment composition to 99 parts of water. It is essential that pH of the composition is less than or equal to 6. The fabric treatment composition preferably comprises an acid other than the fatty acid in order to ensure that pH of the fabric treatment composition is less than or equal to 6. The acid other than fatty acid is preferably from 0.1 % to 20%, more preferably 0.5 to 10% and most preferably from 1% to 5% by weight of the fabric treatment composition.

### Surfactant

The composition may comprise a surfactant. However the surfactant if present, is preferably not greater than 5%, more preferably not greater than 2% and most preferably not greater than 1% by weight of said composition.

### Optional Ingredients

The fabric treatment composition may comprise other optional ingredients including fluorescer, perfume, and preservative.

### The Method of Treating Fabric

The method of treating fabric comprises a step of contacting the fabric with the fabric treatment composition in presence of water.

It is essential the step of contacting the fabric with the fabric treatment composition in presence of water is at a pH less than or equal to 6. The pH may be maintained by adding an acid to the fabric treatment composition. Alternatively, an acid may be added during the step of contacting so as to ensure that the pH during the step of contacting the fabric is less than or equal to 6.

### EXAMPLES

The invention will now be demonstrated with examples. The examples are for the purpose of illustration only and do not limit the scope of the invention in any manner.

### The Method Of Treatment Of Fabric

Fabric treatment compositions were prepared by mixing clay, poydimethylsiloxane (Q2-1607 emulsion from Dow Corning) and fatty acid and adding citric acid solution to adjust pH to 5 unless specified otherwise. The % by weight of polydimethylsiloxane in the composition is given on water-free basis unless specified otherwise. The fabric treatment composition was added to water (1.4 g of the composition in 200 mL of water) to prepare an aqueous suspension. A fabric swatch (size 10 cm X 10 cm) made of desized cotton, polycotton or polyester (all obtained from Bombay Dyeing, India) was dipped in the above suspension. The liquor to cloth ratio of about three was maintained. After 15 minutes of soaking, the fabric swatch was removed from the suspension and dried at 40°C for about 1 hour. The dried swatches were then ironed.

### Evaluation of Hydrophobicity of Fabrics

Contact angle was measured using Kruss Contact Angle Measurement Unit. Fabric swatch (either treated or untreated) was placed and a 20 µL drop of deionized water was placed on the fabric using a syringe. Contact angle was determined using digital photographs captured at interval of 2 seconds for a period of 2 minutes. Fabric was rated as hydrophobic if the contract angle of greater than 90° of the drop was maintained for a period of 2 minutes. Fabric was rated as not hydrophobic if the drop spreaded on the fabric before 2 minutes.

### Effect Of Amount Of Clay:

The fabric treatment compositions are tabulated below. All the fabric treatments were at pH 5. The results of evaluation of hydrophobicity are also tabulated below.

**Table 1: Effect of amount of clay**

| Ex No | Sodium bentonite (% by weight) | Stearic acid (% by weight) | Silicone oil (% by weight) | Clay/F atty acid ratio | Hydrophobicity | | |
|---|---|---|---|---|---|---|---|
| | | | | | cotton | polycotton | polyester |
| 1 | 79 | 16 | 5 | 5 | Y | Y | Y |
| 2 | 70 | 23 | 7 | 3 | Y | Y | Y |
| 3 | 43.5 | 43.5 | 13 | 1 | N | Y | Y |
| A | 28 | 56 | 16 | 0.5 | N | N | Y |

From the results, it is clear that the fabric treatment composition comprising at least 30% clay provides hydrophobicity on cotton, polycotton and polyester swatches whilst the fabric treatment composition comprising less than 30% by weight provides hydrophobicity only on polyester swatches. It can be further seen that the hydrophobicity of treated fabrics improves as the mass ratio of clay to fatty acid in the composition exceeds 1.

### Effect of pH

Fabrics were treated with a composition similar to the composition of Ex No 1 except that myristic acid was used instead of stearic acid. The treatments were carried out at different values of pH as tabulated below. All the experiments were at clay to fatty acid mass ratio of 5. The results of evaluation of hydrophobicity are tabulated below.

**Table 2: Effect of pH during the treatment**

| Ex No | pH | Hydrophobicity on cotton | Hydrophobicity on polycotton | Hydrophobicity on polyester |
|---|---|---|---|---|
| 4 | 3 | Y | Y | Y |
| 5 | 4 | Y | Y | Y |
| 6 | 5 | Y | Y | Y |
| 7 | 6 | Y | Y | Y |
| B | 7 | Y | N | N |

From the results, it is clear that the fabric treatment at a pH of 6 or less than 6 provides hydrophobicity on cotton, polycotton and polyester swatches whilst the fabric treatment at pH greater than 6 provides hydrophobicity only on cotton swatches.

### Effect of Type of Clay

The treatment composition used in Ex No 8 is same as that used in Ex No 1 in all respects except that 1:1 clay was used instead of 2:1 clay. The treatment was at pH of 5. The results of evaluation of hydrophobicity are tabulated below. The results of Ex No 1 are reproduced below for convenience.

**Table 3: Effect of type of clay**

| Ex No | Clay | Hydrophobicity on cotton | Hydrophobicity on polycotton | Hydrophobicity on polyester |
|---|---|---|---|---|
| 1 | Sodium bentonite (2:1 clay) | Y | Y | Y |
| 8 | Kaolinite (1:1 clay) | N | Y | Y |

From the results, it is clear that the fabric treatment composition comprising 2:1 clay provides hydrophobicity on cotton, polycotton and polyester swatches whilst the fabric treatment composition comprising 1:1 clay provides hydrophobicity only on polycotton and polyester swatches.

### Effect Of Type Of Fatty Acid

The treatment compositions were same as those used in Ex No 1 except for the type of fatty acid used, which are given in the table below. All the treatments were at pH of 5. The results of evaluation of hydrophobicity are tabulated below.

**Table 4: Effect of type of fatty acid**

| Ex No | Fatty acid | Hydrophobicity on cotton | Hydrophobicity on polycotton | Hydrophobicity on polyester |
|---|---|---|---|---|
| 9 | Lauric acid | Y | Y | Y |
| 10 | Palmitic acid | Y | Y | Y |
| 11 | Oleic acid | N | Y | Y |

From the results, it is clear that the fabric treatment composition comprising saturated fatty acid provides hydrophobicity on cotton, polycotton and polyester swatches whilst the fabric treatment composition comprising unsaturated fatty acid provides hydrophobicity only on polycotton and polyester swatches.

### Effect Of Amount Of Fatty Acid In The Composition

The fabric treatment compositions comprised stearic acid, silicone and sodium bentonite as tabulated below. All the treatments were at pH of 5. The results of evaluation of hydrophobicity are tabulated below.

**Table 5: Effect of amount of fatty acid in the composition**

| Ex No | Bentonite (% by weight) | Stearic acid (% by weight) | Silicone oil (% by weight) | Hydrophobicity | | |
|---|---|---|---|---|---|---|
| | | | | cotton | polycotton | polyester |
| 12 | 86 | 9 | 5 | Y | Y | Y |
| 13 | 90 | 4.5 | 5.5 | Y | Y | Y |
| C | 93 | 2 | 5 | N | Y | Y |

It can be seen that the ompositions comprising at least 5% fatty acid by weight provide hydrophobicity on all substrates including cotton.

### Evaluation Of Stain Repellency

### Staining of fabrics

Three types of stains were used, prepared using following method.
1. Mud stain - 1g red soil obtained locally from Bangalore India (average particle size 180 micron,) was suspended in 200 mL deionized water.
2. Ketchup stain - 5 mL Kissan® (Hindustan Unilever Limited) tomato sauce was mixed in 200 mL deionized water
3. Tea stain - 3 Taj Mahal® (Hindustan Unilever Limited) tea-bags (6 g total) were dipped in 300 mL deionized water maintained at 80 °C for 20 minutes.

1 mL of above staining solution was poured drop by drop (from a height of 0.5 cm) using a micropipette over treated (according to Ex No 1) and untreated fabric swatch placed on a flat surface inclined at 40° from the horizontal. The behaviour of drops was observed to vary between two extremes. In some cases the drop of the staining solution rolled off from the fabric and in some cases the staining solution spread completely on the fabric instead of rolling off. The resulting staining of fabric was evaluated by a panel of 7 persons, who graded the staining on a scale of 0 to 5, with a score of 0 indicating no staining and a score of 5 indicating maximum staining. A low score indicates high stain repellency and vice versa. The results of evaluation of stain repellency are tabulated below.

**Table 6: Stain repellency of treated fabrics**

| | Mud | | Tea | | Ketchup | |
|---|---|---|---|---|---|---|
| Fabric type | Treated | Untreated | Treated | Untreated | Treated | Untreated |
| Cotton | 0.2 | 4.4 | 1.1 | 3.9 | 1.3 | 3.9 |
| Polycotton | 1.0 | 4.4 | 0.9 | 3.8 | 0.1 | 3.6 |
| Polyester | 2.5 | 4.4 | 1.6 | 3.3 | 1.8 | 3.2 |

From the results, it can be seen that the fabrics treated by the method and the composition of the present invention have relatively higher stain-resistance.

It will be appreciated that the method and composition of fabric treatment according to the present invention render the fabrics relatively more hydrophobic and impart relatively better stain-resistance to the fabric.

## Claims

1. A fabric treatment composition comprising clay, silicone oil, and fatty acid, **characterized in that**:
i) the composition comprises at least 30% by weight of clay, and
ii) pH of the composition is less than or equal to 6, wherein by the pH of the fabric treatment composition is meant the pH of a mixture obtained by adding 1 part of the fabric treatment composition to 99 parts of water.

2. A fabric treatment composition as claimed in claim 1 wherein said clay is a 2:1 clay.

3. A fabric treatment composition as claimed in claim 1 or claim 2 wherein said fatty acid is a saturated fatty acid.

4. A fabric treatment composition as claimed in any one of the preceding claims wherein said fatty acid is from 5% to 50% by weight of the composition.

5. A fabric treatment composition as claimed in any one of the preceding claims wherein the mass ratio of clay to fatty acid is greater than 1.

6. A fabric treatment composition as claimed in any one of the preceding claims wherein said clay is from 30% to 90% by weight of the composition.

7. A fabric treatment composition as claimed in any one of the preceding claims wherein said silicone oil Is from 3% to 50% by weight of the composition.

8. A fabric treatment composition as claimed in any one of the preceding claims wherein the composition comprises a surfactant in an amount not greater than 5% by weight of said composition.

9. A fabric treatment composition as claimed in any one of the preceding claims comprising from 0.1% to 20% by weight an acid other than the fatty acid.

10. A method of treating fabric **characterized in that** it comprises a step of conlacting the fabric with the fabric treatment composition as claimed in any one of the claims 1-9 in presence of water.

## Patentansprüche

1. Gewebebehandlungszusammensetzung, die Ton, Silikonöl und Fettsäure umfasst, **dadurch gekennzeichnet, dass**:
i) die Zusammensetzung wenigstens 30 Gew.-% Ton umfasst und
ii) der pH der Zusammensetzung kleiner als oder gleich 6 ist, wobei mit dem pH der Gewebebehandlungszusammensetzung der pH eines Gemisches gemeint ist, das durch Zusetzen von 1 Teil der Gewebebehandlungszusammensetzung zu 99 % Wasser erhalten wird.

2. Gewebebehandlungszusammensetzung, wie sie in Anspruch 1 beansprucht ist, wobei der Ton ein 2:1 Ton ist.

3. Gewebebehandlungszusammensetzung, wie sie in Anspruch 1 oder Anspruch 2 beansprucht ist, wobei die Fettsäure eine gesättigte Fettsäure ist.

4. Gewebebehandlungszusammensetzung, wie sie in einem der vorangehenden Ansprüche beansprucht ist, wobei die Fettsäure 5 bis 50 Gew.-% der Zusammensetzung ausmacht.

5. Gewebebehandlungszusammensetzung, wie sie in einem der vorangehenden Ansprüche beansprucht ist, wobei das Massenverhältnis von Ton zu Fettsäure größer als 1 ist.

6. Gewebebehandlungszusammensetzung, wie sie in einem der vorangehenden Ansprüche beansprucht ist, wobei der Ton 30 bis 90 Gew.-% der Zusammensetzung ausmacht.

7. Gewebebehandlungszusammensetzung, wie sie in einem der vorangehenden Ansprüche beansprucht ist, wobei das Silikonöl 3 bis 50 Gew.-% der Zusammensetzung ausmacht.

8. Gewebebehandlungszusammensetzung, wie sie in einem der vorangehenden Ansprüche beansprucht ist, wobei die Zusammensetzung ein Tensid in einer Menge von nicht größer als 5 Gew.-% der Zusammensetzung umfasst.

9. Gewebebehandlungszusammensetzung, wie sie in einem der vorangehenden Ansprüche beansprucht ist, die 0,1 bis 20 Gew.-% einer anderen Säure als die Fettsäure umfasst.

10. Verfahren zur Gewebebehandlung, **dadurch gekennzeichnet, dass** es einen Schritt des In-Kontakt-Bringens des Gewebes mit der Gewebebehandlungszusammensetzung, wie sie in einem der Ansprüche 1 bis 9 beansprucht ist, in Gegenwart von Wasser umfasst.

## Revendications

1. Composition de traitement de tissu comprenant de l'argile, une huile de silicone et un acide gras, **caractérisée en ce que** :
i) la composition comprend au moins 30 % en poids d'argile, et
ii) le pH de la composition est inférieur ou égal à 6, où par le pH de la composition de traitement de tissu, il est signifié le pH d'un mélange obtenu par l'addition de 1 partie de la composition de traitement de tissu pour 99 parties d'eau.

2. Composition de traitement de tissu selon la revendication 1, dans laquelle ladite argile est une argile 2:1.

3. Composition de traitement de tissu selon la revendication 1 ou la revendication 2, dans laquelle ledit acide gras est un acide gras saturé.

4. Composition de traitement de tissu selon l'une quelconque des revendications précédentes, dans laquelle ledit acide gras représente de 5 % à 50 % en poids de la composition.

5. Composition de traitement de tissu selon l'une quelconque des revendications précédentes, dans laquelle le rapport massique de l'argile sur l'acide gras est supérieur à 1.

6. Composition de traitement de tissu selon l'une quelconque des revendications précédentes, dans laquelle ladite argile représente de 30 % à 90 % en poids de la composition.

7. Composition de traitement de tissu selon l'une quelconque des revendications précédentes, dans laquelle ladite huile de silicone représente de 3 % à 50 % en poids de la composition.

8. Composition de traitement de tissu selon l'une quelconque des revendications précédentes, dans laquelle la composition comprend un surfactant dans une quantité qui n'est pas supérieure à 5 % en poids de ladite composition.

9. Composition de traitement de tissu selon l'une quelconque des revendications précédentes, comprenant de 0,1 % à 20 % en poids d'un acide autre que l'acide gras.

10. Procédé de traitement de tissu **caractérisé en ce qu'**il comprend une étape consistant à mettre en contact le tissu avec la composition de traitement de tissu selon l'une quelconque des revendications 1 à 9 en présence d'eau.
